

## UNITED STATES PATENT OFFICE

2,393,488

BERYLLIUM ALLOY STEELS AND ARTICLES  
OF MANUFACTURE PRODUCED THERE-  
FROMEnrique G. Touceda, Loudonville, and Ralph P.  
De Vries, Menands, N. Y., assignors to Alle-  
gheny Ludlum Steel Corporation, a corporation  
of PennsylvaniaNo Drawing. Application July 28, 1942,  
Serial No. 452,636

2 Claims. (Cl. 75—126)

The present invention relates to beryllium-containing alloy steels and to products produced therefrom by casting, forging and rolling.

Magnet steels are characterized by the fact that they retain a large proportion of the magnetism induced in them when placed in a magnetic field. By hardening them as much as possible their retentivity is greatly increased. Steels containing chromium in various amounts up to about 6% have been employed for magnets due to their relatively high retentivity. It is very difficult, however, to produce chromium magnet steels containing chromium in the indicated range in rolled form with a coercive force ( $H_c$ ) of 60 or more and in any event it is essential that special precautions be taken in the processing and hardening thereof to produce optimum coercive force values. In addition to this, such magnet steels do not have a BH value as high as is desired and these facts coupled with the necessity of using relatively high carbon—at least about .90% and the lack of hardness and ductility as determined by Rockwell Cone hardness tests and transverse bending tests, respectively, have left the chromium magnet steel situation in a relatively unsatisfactory condition. Therefore, the industry is still seeking for improved magnet steels which are not only simple and inexpensive to produce but which have better magnetic and physical characteristics than those heretofore available.

One of the objects of our present invention is to produce magnet steels which overcome the defects and disadvantages outlined above and which have additional advantages by virtue of their unusual composition.

Another object of our invention is to produce magnet steels modified by the incorporation therein of a small amount of beryllium and characterized by exceptionally desirable magnetic and physical properties.

A further object of our invention is to produce magnet steels which, in addition to iron and the usual impurities in common amounts, contain chromium and a relatively small amount of carbon and beryllium in approximately the amounts hereinafter specified.

A still further object of our invention is to produce a beryllium alloy steel suitable for magnets and other commercial articles of manufacture and which, as hereinafter more fully set forth, is characterized by excellent magnetic properties, by greater hardness and strength and by better fluidity when in the molten state than known magnet steels.

A still further object of our invention resides

in the production of magnet steels and steels adapted for various other commercial products which are especially characterized by the fact that they contain, in addition to iron and the usual impurities in common amounts, a carbon content which may range from about .10% to about 1.25%, a chromium content which may range from about 1% to about 8% and a small amount of beryllium which is always under 1% and which preferably ranges from about .03% to about .7%.

Other and further objects and advantages will be understood by those skilled in this art or will be apparent or pointed out below.

15 Our present invention is predicated upon the discovery that markedly superior properties can be imparted to alloy steels by the incorporation therein of a small amount of beryllium (less than 1%). This beryllium addition confers new and 20 highly valuable magnetic properties on our compositions thus rendering them particularly adapted for employment in the production of permanent magnets. The beryllium addition has other unexpected and valuable effects and in particular such are manifested by the ability materially to reduce the amount of carbon employed, thus avoiding the processing difficulties accompanying the use of relatively high carbon contents; by the imparting of materially greater 25 hardness, as determined, for example, by Rockwell Cone hardness tests; by increasing the strength of the compositions, as determined by transverse bending tests, and hence by increased ductility and by endowing the material when in 30 the molten state with a substantially improved fluidity, thus facilitating casting operations.

As above indicated, our present invention involves alloy steels which, in addition to iron and the usual impurities in common amounts, contain 35 certain percentages of carbon, chromium and beryllium. In the practice of our invention, carbon may be incorporated in our new steels to the extent of from about .10% to about 1.25% but in those cases in which carbon is employed for use 40 in magnet steels it is essential that it be present in the amount of at least .70% and may range from that value up to and including the maximum specified. The chromium content of our new alloy steels ranges from about 1% to about 8%. 45 The present day chromium magnet steels, while generally satisfactory and extensively utilized, are difficult to produce with optimum magnetic characteristics and, therefore, our present invention is concerned with bringing about an improvement in connection with this disadvantage. The

beryllium content of our new alloy steels is always less than 1% and preferably ranges in amount from about .03% to about .7%. Our new steels may optionally contain from about .10% to about .50% of silicon and of manganese. The usual impurities are generally the metalloids phosphorus and sulfur and these are present in common amounts. Iron constitutes substantially the entire balance.

Beryllium alloy steels as defined above possess superior magnetic properties. Similar steels containing no beryllium can be produced from the as rolled condition after hardening with a coercive force ( $H_c$ ) as high as about 60 only with great difficulty, whereas in marked and direct contrast thereto our new steels can be readily produced from the as rolled condition after hardening with coercive force values considerably above 60 without taking any special precautions in the processing and hardening of such steels. This is not only highly advantageous in connection with the use of these compositions but represents very definite economic and commercial advantages as well.

Table I, which follows, is illustrative of the improved magnetic properties characteristic of our new beryllium alloy steels:

Table I

| Melt # | C    | Cr   | Si   | Mn   | Mo  | W   | Be   | As quenched hardness cone Rockwell | Temperature and condition | $B_{max.}$ | $B_r$ | $H_c$ | BH      |
|--------|------|------|------|------|-----|-----|------|------------------------------------|---------------------------|------------|-------|-------|---------|
| 135-B  | 0.93 | 3.69 | 0.16 | 0.39 |     |     | None | 62                                 | (As rolled)               | 11,491     | 8,383 | 59    | 494,000 |
| 135-B  | .93  | 3.69 | .16  | .39  |     |     | None | 62                                 | 1,550—oil                 | 11,882     | 8,548 | 60.3  | 516,000 |
| M-32   | 1.07 | 3.72 | .31  | .46  |     |     | 0.10 | 62                                 | 1,550—oil                 | 12,124     | 8,652 | 63.0  | 538,000 |
| M-32   | 1.07 | 3.72 | .31  | .46  |     |     | .10  | 61                                 | 1,550—oil                 | 11,446     | 8,196 | 66.0  | 541,000 |
| M-42   | .90  | 3.70 | .33  | .32  |     |     | .20  | 61                                 | 1,550—oil                 | 12,400     | 8,714 | 67.2  | 536,000 |
| M-42   | .90  | 3.70 | .33  | .32  |     |     | .20  | 63                                 | 1,550—oil                 | 11,492     | 8,135 | 71.6  | 533,000 |
| M-43   | .91  | 2.18 | .28  | .34  |     |     | .20  | 62                                 | 1,550—oil                 | 12,078     | 8,583 | 68.6  | 539,000 |
| M-43   | .91  | 2.18 | .28  | .34  |     |     | .20  | 65                                 | 1,550—oil                 | 11,649     | 8,357 | 69.0  | 576,000 |
| M-47   | .91  | 2.09 | .31  |      |     |     | .10  | 62                                 | 1,550—oil                 | 12,265     | 8,644 | 62.8  | 543,000 |
| M-47   | .91  | 2.09 | .31  |      |     |     | .10  | 61                                 | 1,550—oil                 | 11,106     | 7,702 | 64.0  | 493,000 |
| M-48   | .89  | 3.83 | .45  |      |     |     | .20  | 61                                 | 1,550—oil                 | 12,009     | 8,327 | 67.4  | 561,000 |
| M-48   | .89  | 3.83 | .45  |      |     |     | .20  | 65                                 | 1,550—oil                 | 11,216     | 7,874 | 72.0  | 566,000 |
| M-56   | .97  | 6.94 |      |      |     |     | .20  | 67                                 | 1,550—oil                 | 12,430     | 8,895 | 66.0  | 594,000 |
| M-56   | .97  | 6.94 |      |      |     |     | .20  | 67                                 | 1,600—oil                 | 11,178     | 7,765 | 64.5  | 501,000 |
| M-57   | .95  | 2.18 |      |      |     |     | .20  | 63                                 | 1,550—oil                 | 11,649     | 8,335 | 70.0  | 594,000 |
| M-57   | .95  | 2.18 |      |      |     |     | .20  | 66                                 | 1,600—oil                 | 10,649     | 7,559 | 72.0  | 545,000 |
| M-58   | .99  | 3.65 |      |      |     |     | .18  | 60                                 | 1,550—oil                 | 12,015     | 8,389 | 63.5  | 581,000 |
| M-58   | .99  | 3.65 |      |      |     |     | .18  | 63                                 | 1,600—oil                 | 12,708     | 8,893 | 64.0  | 570,000 |
| M-59   | .98  | 3.77 |      |      |     |     | .25  | 63                                 | 1,550—oil                 | 12,443     | 8,894 | 64.0  | 570,000 |
| M-59   | .98  | 3.77 |      |      |     |     | .25  | 66                                 | 1,600—oil                 | 11,171     | 8,050 | 68.0  | 547,000 |
| M-53   | .85  | 2.12 | .35  | .14  | .79 | .45 |      | 62                                 | 1,550—oil                 | 10,418     | 7,371 | 73.7  | 543,000 |
| M-53   | .85  | 2.12 | .35  | .14  | .79 | .45 |      | 62                                 | 1,550—oil                 | 10,529     | 7,427 | 73.7  | 547,000 |
| T-233  | .89  | 1.94 |      |      | .47 | .50 |      | 66                                 | (As forged)               | 11,662     | 8,352 | 62.0  | 518,000 |

Cross section of rolled and hardened bars=1 $\frac{1}{4}$ " x 36".

This table sets forth pertinent and important data concerning several compositions responding to our present invention as well as some compositions which have been included for comparative purposes. The first column in the table serves to identify the individual compositions tested. The next columns give the analyses of those compositions. The next succeeding column sets forth the Rockwell Cone hardness of each composition in the as quenched condition. The next column sets forth the quenching and/or other conditions of each composition from which the magnetic properties in the four right-hand columns of the Table were derived. The heading  $B_{max.}$  indicates the maximum number of magnetic lines of force induced in each test piece under the test conditions,  $B_r$  indicates residual induction after reversal of the magnetic field and  $H_c$  indicates coercive force. The last column, with the heading BH, is the product of the residual induction ( $B_r$ ) and the coercive force ( $H_c$ ), the values of BH being given as approximations only.

BH value is considered to be the best criterion of the strength of a permanent magnet. It will be noted from the table that whereas the conventional chrome magnet steel 135-B has a BH value of about 500,000, composition M-43 responding to our present invention and containing about 1 $\frac{1}{2}$  less chromium but with a .20% beryllium, has a BH value of nearly 60,000. The BH values of the beryllium-containing compositions are considerably greater than those without beryllium and the coercive force of such compositions is in every case above 60, some of the coercive forces running above 70. Attention is also directed to the fact that composition M-53 which, in addition to 2.12% of chromium, contains .45% of beryllium and .79% of tungsten, has a very good coercive force of almost 74 and a BH value averaging about 545,000, but nevertheless it is not as strong magnetically as composition M-57 which not only contains no tungsten but which also contains less than  $\frac{1}{2}$  as much beryllium. The M-53 composition is, however, appreciably stronger magnetically than composition T-233 which contains preferred amounts of molybdenum and tungsten but which has no beryllium content.

In producing the highest quality permanent magnet steels in accordance with prior practices,

it has been considered essential to have at least .90% of carbon present. In connection with our present invention we have further discovered that the presence of beryllium even in very small quantities reduces the carbon requirements down to a minimum of about .70% while still making it possible to produce steels having magnetic values at least equal to those of the beryllium-free chromium steels with the higher carbon contents. This is a distinct commercial advantage because it permits both the steels themselves and the permanent magnets made from such steels to be produced more easily and inexpensively without going through the precautionary measures which must be carried out in producing the standard chromium magnet steels.

Table I also shows that the compositions which contain beryllium are on the whole harder than those without beryllium as determined by Rockwell Cone hardness tests in the as quenched state. Coercive force has frequently been used as a measure of hardness and from the table it will

be observed that the higher coercive forces are usually associated with the higher hardness values. It is thus possible to obtain a hardness value in the range of 62-64 Cone Rockwell on chromium steels which contain no essential elements other than about 1% of carbon, but the beryllium-containing chromium steels exhibit generally better hardness values and in some instances show hardness values ranging as high as 67 Cone Rockwell. These beryllium steels are, therefore, useful for ball-bearing steels which are subjected to high pressures and high speeds as well as for projectiles and many other purposes where ordinary chromium steels do not provide that extra necessary margin of hardness and strength which is requisite for many usages.

In order to determine the direct effect of varying percentages of beryllium a number of compositions were produced which were substantially identical except for the beryllium content. Several such compositions and the important properties thereof are set forth in Table II, which follows:

Table II

| Melt<br># | C    | Cr   | Si  | Mn  | Be   | As cast<br>cone<br>Rockwell | As<br>quenched<br>1550° F. oil<br>cone<br>Rockwell | Magnetic properties |                |                |         |
|-----------|------|------|-----|-----|------|-----------------------------|----------------------------------------------------|---------------------|----------------|----------------|---------|
|           |      |      |     |     |      |                             |                                                    | B <sub>max.</sub>   | B <sub>r</sub> | H <sub>c</sub> | BH      |
| M-64----- | 1.00 | 2.16 | .20 | .06 | 0.20 | 60                          | 66                                                 | 11,300              | 8,119          | 65.2           | 529,000 |
| M-65----- | .98  | 2.22 | .25 | .07 | .40  | 49                          | 66                                                 | 10,419              | 7,493          | 68.5           | 514,000 |
| M-66----- | 1.01 | 2.22 | .19 | .07 | .60  | 54                          | 62                                                 | 10,112              | 6,919          | 65.0           | 450,000 |
| M-67----- | .99  | 2.16 | .08 | .06 | None | 46                          | 56                                                 | 11,798              | 7,891          | 51.0           | 403,000 |

Cross section of cast and hardened bars  $1\frac{1}{4}''$  x  $5\frac{1}{16}''$ .

Referring to this table it will be appreciated that the compositions there included range from 0% beryllium (M-67) to .60% beryllium (M-66). These compositions were tested in the as cast condition. In each instance a straight bar  $1\frac{1}{4}''$  x  $\frac{1}{8}''$  was cast in a permanent graphite mold. The cast bar containing .20% beryllium has the highest BH value and possessed the greatest hardness in the as cast condition, whereas the beryllium-free composition showed up poorest in both respects. As quenched in oil at 1550° F., the beryllium-free composition has the lowest Rockwell Cone hardness value and the .20% and .40% beryllium compositions show the best hardness values. Attention is further directed to the fact that the beryllium-free composition M-67 does not approach in the cast condition the magnetic values obtainable in the rolled and hardened state as illustrated in Table I.

Beryllium steels responding to the present invention possess a greater fluidity when in the molten state than beryllium-free steels. In one experiment, molten beryllium steel was bottom-poured into a mold having a  $\frac{1}{2}$ " diameter and rose in that mold to a height of 10", whereas under the same conditions beryllium-free compositions rose to a height 3" to 4" less. This result is independent of the casting temperature. The improved fluidity is naturally a decided advantage in making castings by any method and therefore for many purposes our alloy steels may be cast and hardened to high hardness values and when they are to be used for magnets they have much better properties than rolled chromium magnet steels. These beryllium steels both in the as cast and in the as rolled condition retain their hardness much longer after drawing to higher temperatures than do the straight chromium steels without beryllium. This prop-

erty of hardness retention has a valuable application to ball-bearing and races.

In Table III a further interesting and important property (the strength) of cast chromium beryllium steels is delineated:

| Melt # | C    | Cr   | Si   | Mn   | Be   | Bend           | F p. s. i. | Hardness Rockwell C |
|--------|------|------|------|------|------|----------------|------------|---------------------|
| 10     |      |      |      |      |      |                |            |                     |
| M-66   | 1.01 | 2.22 | 0.19 | 0.07 | 0.60 | <i>Degrees</i> |            |                     |
| M-65   | .98  | 2.22 | .25  | .07  | .40  | 0              | 92,000     | 64/65               |
| M-64   | 1.00 | 2.16 | .20  | .08  | .20  | 0              | 67,000     | 64/65               |
| M-67   | .99  | 2.16 | .08  | .06  | None | 0              | 59,000     | 64/66               |
|        |      |      |      |      |      | 0              | 44,000     | 63/64               |

1 1/4" x 5/8" = 1550° F. oil.

These four steels (M-64 to M-67, inclusive) were all quenched in oil from the same temperature and were all then tested in transverse. 20 The expectation was that fully-hardened steels would break prematurely and would consequently show wide variations in strength due to lack of ductility needed to develop their full strength.

Table II

| Melt<br># | C    | Cr   | Si  | Mn  | Be   | As cast<br>cone<br>Rockwell | As<br>quenched<br>1550° F. oil<br>cone<br>Rockwell | Magnetic properties |                |                |         |
|-----------|------|------|-----|-----|------|-----------------------------|----------------------------------------------------|---------------------|----------------|----------------|---------|
|           |      |      |     |     |      |                             |                                                    | B <sub>max.</sub>   | B <sub>r</sub> | H <sub>c</sub> | BH      |
| M-64----- | 1.00 | 2.16 | .20 | .06 | 0.20 | 60                          | 66                                                 | 11,300              | 8,119          | 65.2           | 529,000 |
| M-65----- | .98  | 2.22 | .25 | .07 | .40  | 49                          | 66                                                 | 10,419              | 7,493          | 68.5           | 514,000 |
| M-66----- | 1.01 | 2.22 | .19 | .07 | .60  | 54                          | 62                                                 | 10,112              | 6,919          | 65.0           | 450,000 |
| M-67----- | .99  | 2.16 | .08 | .06 | None | 46                          | 56                                                 | 11,798              | 7,891          | 51.0           | 403,000 |

The results shown in the table, however, prove that the strength actually developed in the transverse bending tests is beneficially influenced in proportion to the beryllium content. In other words, the composition with the highest beryllium content gave the highest test results and the lowest test results occurred with respect to that composition which contained no beryllium. As to the intermediate compositions, M-64 with a .20% beryllium is materially better than M-67 without beryllium but M-65 with a .40% beryllium was even better than M-64.

50 It will be observed and appreciated from what has preceded that the incorporation of even a very small amount of beryllium has a remarkable effect upon the properties of the alloy steel to which the same has been added. A beryllium content of as little as about .03% is effective, 55 the results differing primarily in their extent and intensity from those compositions containing larger percentages of beryllium. For many purposes the beryllium content need not be more than .1 or .2% but the particular amount of beryllium which should be employed depends upon the intended use of any given composition and therefore upon the properties which that use predetermines. As will be noted, beryllium has the capacity to increase the hardness and 60 strength of alloy steels such as the chromium alloy steels, to impart unusually excellent magnetic properties to compositions which are used for permanent magnets and other magnetic equipment, to enable the amount of carbon to be 65 reduced with consequent elimination of the precautionary measures ordinarily required for higher carbon contents and to impart to the compositions a considerably better fluidity when in the molten state, thus facilitating and expediting 70 casting operations of all types. The new, use- 75

ful and unexpected results of incorporating small percentages of beryllium (under 1%) in alloy steels in accordance with our present invention could not have been predicted on the basis of existing knowledge. The practice of our present invention not only produces products which are superior and commercially advantageous but it also results in improvements in production operations and technique.

The foregoing is intended as illustrative and not as limitative and, without departing from the scope and principles hereof, we may resort to various additions, omissions, substitutions and modifications. The invention is rather that defined by the appended claims.

Having thus described our invention, what we claim as new and desire to secure by Letters Patent is:

1. A permanent magnet composed of an alloy

steel consisting of from about 1 to about 8% chromium, from about .10 to about 1.25% carbon and beryllium from about .03 to about .70% with the balance all iron except for the usual impurities in common amounts and characterized by a BH value of about 600,000 by a coercive force above 60 and by a Rockwell hardness value greater than a magnet made from a similar alloy steel without beryllium within such range.

2. A magnet cast from an alloy consisting of approximately 1.00% carbon, chromium within the range of from about 2.00% to about 4.00%, beryllium within the range of from about 0.03% to about 1.00%, silicon and manganese each within the range of from about 0.10% to about 0.50% and the remainder iron except for usual impurities in common amounts.

ENRIQUE G. TOUCEDA.  
RALPH P. DE VRIES.